

Dec. 20, 1938.

C. V. CANNING

2,140,506

STENCIL SHEET

Filed Sept. 29, 1932

Fig. 1.

Composition of Rubber, Coumarone  
Resin and Mineral Oil



Fig. 2.



Fig. 3.

Composition of Gum Chicle, Rubber,  
(Paraffin Wax and Resin



Inventor

C. V. Canning

By

Foster & Codier

Attorney

## UNITED STATES PATENT OFFICE

2,140,506

## STENCIL SHEET

Charles V. Canning, New York, N. Y., assignor to  
 Sweets Laboratories, Inc., New York, N. Y., a  
 corporation of New York

Application September 29, 1932, Serial No. 635,428

8 Claims. (Cl. 41—38.6)

The present invention relates to stencil sheets, and has for its object to produce a stencil sheet which shall be durable, capable of giving sharp impressions, when used on duplicating machines, and which will remain unaltered in storage for a long time, and will be economical to manufacture and convenient to use.

Sheets are well known, for use as stencil sheets, which have as a base a sheet of relatively porous strong paper such as Yoshino paper, having a coating which is readily perforated by means of the type of a typewriter (the ribbon usually being pulled back out of the way during such operation) and also which will be perforated by means of a stylo. Such sheets are used on the duplicating machine such as the Neostyle and others, for producing many copies of a letter, or other subject matter of which copies may be desired.

In accordance with the present invention I have found that highly suitable stencil sheets may be prepared from paper such as Yoshino or other paper of similar characteristics, by coating the same on one or both sides with a composition containing rubber, coumarone resin and a mineral or other oil acting as a softening agent. The proportions of the materials to be employed can be varied considerably, but the following proportions have been found in practice to be very satisfactory:

|                                        | Per cent |
|----------------------------------------|----------|
| Rubber (unvulcanized)                  | 28.5     |
| Coumarone M. P. 140 degrees centigrade | 60       |
| Coumarone M. P. 63 degrees centigrade  | 9        |
| Mineral oil                            | 2.5      |

The above composition can be dissolved in a suitable solvent, and any desired coloring matter can be added to the solution or to the material before dissolving the same in the solvent, after which the paper may be dipped into the solution or contacted with the upper surface of the solution in such a way as to coat one side only of the paper with the solution. Then the solvent is evaporated, leaving the mixture consisting essentially of rubber, coumarone resin and mineral oil, firmly adhering to the paper. Such a sheet may be applied in the usual manner to the backings which are commonly used in the art, and will be found to have the desired degree of flexibility and the properties above referred to. The oil used on this formula may be a high viscosity lubricating oil, e. g. automobile motor oil.

In some cases it may be advisable to coat the paper on both sides with the said composition, and the coating on the reverse side being very thin. Usually coating on one side is better.

Another formula for a coating composition for this purpose, which has been found to be highly satisfactory is the following:

|                     | Per cent |
|---------------------|----------|
| Gum chicle          | 50       |
| Unvulcanized rubber | 15       |
| Paraffin wax        | 20       |
| Coumarone resin     | 10       |

In the first formula, instead of the unvulcanized rubber, it is possible to also employ other rubbery materials, preferably in an unvulcanized condition. In place of the coumarone resin above referred to, other resins (natural or synthetic) can sometimes be substituted for all or a portion of the coumarone resin. Resinous rubbers such as Pontianak can be used, in place of some or all of the coumarone resin. I have in the first above formula used two different grades of coumarone resin, one being of a relatively high melting point such as 140° C., and the other being of a much lower melting point, say 63° C. It will be understood that various blends of hard and soft coumarone resin, with or without various other resins can be employed, or a resin having an intermediate melting point. Such materials and mixtures are hereinafter included in the term resin. In some cases it is advisable to also add to the first formula, a small proportion of a wax such as beeswax, paraffine wax, Japan wax or a mixture of these. Stearin or other fats can also be used, and liquid fatty oils can be used. The latter can replace the mineral oil used in the above formula, and the waxes and fats can be substituted for a part of the coumarone resin, for example can be substituted for the low melting point coumarone resin referred to in the above formula. These substances like the mineral oil, also act as softening agents, and are hereinafter included in the term "softener".

In the second formula, also, the substitutions as referred to, can be made. It is also possible to use rubbery material which also contains a considerable amount of resins, (as a substitute for the resin and a part of the rubber), for example Pontianak or Jelutong. Paraffin wax is mentioned in this formula. In place of all or part of the same, I can employ hard tallow, hard hydrogenated oil. The term "oily material" is intended to include such substances. In place of the coumarone resin, various other synthetic resins and/or natural resins, or mixtures thereof can be used. Various inks or dyes or coloring agents can be added to either of these formulas. Pontianak and Jelutong are rubbery materials from certain shrubs growing in Borneo, Malay

Peninsula and Sarawak, and these contain very large percentages (75 to 85%) of natural resins, and small amounts (10-20% or so) of rubber (on the dry basis). They may contain, in their 5 crude state, as imported, substantial percentages of water, and the said materials are both subject to fermentation.

The solvents applicable for this purpose are carbon tetrachloride or ethylene dichloride or 10 similar rubber solvents, ethylene dichloride being recommended due to the fact that the ink coloring used is dissolved more satisfactorily in it. The proportions may be approximately 3 or 4 parts of solvents to one part of composition.

The coating of both sides of the sheet is not necessary nor generally advisable as it would be apt to make the finished stencil hard to cut through. Furthermore, coating on one side is all 15 that is necessary to make a satisfactory stencil.

20 The rubber can be first roll-milled for 10 to 30 minutes more or less. Then the coumarone resin is blended into the rubber, which can conveniently be done on the roller mill. This mixture can then be incorporated with the other ingredients, either 25 on a roller mill or in a steam-heated mixing kettle having stirring arms or paddles. The partial breaking down of the rubber, as produced on the roller mill, considerably improves the consistency of the mass. The ink or color can be added in the 30 mixing kettle, and obviously any desired color can be employed.

It will be understood that one company may make up and sell the compositions, (with or without the solvent and/or color) and the coating operation (with or without dissolving the composition in a solvent and adding the color) can be performed by another company.

In the annexed drawing I have shown diagrammatically sections of three modifications. In Fig. 40 1 is shown paper carrying the composition on one side only (and naturally the paper will be itself impregnated with the composition). In Fig. 2, I have shown the coating applied to both sides of the paper, the coating on one side here represented 45 as the top being thick, whereas the coating on the other side (here represented as the bottom) being shown thin. Fig. 3 is another modification, as in the second example given.

I am aware that heretofore it has been proposed to employ proteins (including gelatin and 50 glue) or cellulose esters (including nitrocellulose

and cellulose acetate) as the basis of coating compositions for making stencils. I am aware also that it has been proposed to add a modifying agent to modify and alter the normal properties of such proteins and cellulose esters. However I do not employ as the basis of my coating compositions, either proteins or cellulose esters, and the term "protein-free" in certain of the claims of this case is intended to limit the coating composition to coatings which do not contain 10 proteid or protein materials of the type of gelatin or glue.

I claim:—

1. A stencil sheet comprising a paper sheet, carrying a composition comprising unvulcanized 15 rubber, coumarone resin and an oil which will act as a softening agent for such composition.

2. A stencil sheet which consists of paper coated with a composition comprising rubber, high melting point coumarone resin, low melting point 20 coumarone resin, and mineral oil.

3. A stencil sheet which consists of paper coated with a composition comprising about 28.5 parts of unvulcanized rubber, about 60 parts of high melting point coumarone resin, about 9 parts of low 25 melting point coumarone resin and about 2.5 parts of mineral oil.

4. A stencil sheet coated with a composition which consists essentially of plastic non-brittle material selected from the group consisting of 30 rubber and resinous rubber, wax and resin.

5. A stencil sheet coated with a composition which consists essentially of a blend of chicle, rubber and resin, with an oily material.

6. A stencil sheet coated with a composition 35 which is composed essentially of a blend of a plastic non-brittle material selected from the group consisting of rubber and resinous rubber, a resin and a softener.

7. A stencil sheet coated with a composition 40 which is composed essentially of a blend of a plastic non-brittle material selected from the group consisting of rubber and resinous rubber, a resin and an oily material to act as a softening agent.

8. A stencil sheet coated with a composition which is composed essentially of a blend of a plastic non-brittle material selected from the group consisting of rubber and resinous rubber, a resin and a wax to act as a softening agent. 45

CHARLES V. CANNING. 50